

Dec. 23, 1941.

J. EGGERT ET AL

2,267,089

COLOR PHOTOGRAPHY

Filed Dec. 2, 1936

Fig. 1.



Fig. 2.



Inventors,  
John Eggert  
Gerd Heymer

BY

Nutz and Joslin  
THEIR ATTORNEYS

## UNITED STATES PATENT OFFICE

2,267,089

## COLOR PHOTOGRAPHY

John Eggert, Leipzig, and Gerd Heymer, Wolfen,  
Germany, assignors, by mesne assignments, to  
General Aniline & Film Corporation, New  
York, N. Y., a corporation of Delaware

Application December 2, 1936, Serial No. 113,827  
In Germany December 7, 1935

4 Claims. (Cl. 95—2)

The present invention relates to the production of photographic multi-color pictures.

One of its objects is a photographic material producing multi-color component images. Another object is a process of producing multi-color component images. Further objects will be seen from the detailed specification following hereafter.

In the production of three-color components for color photography it has been proposed in U. S. Patent 2,210,146 of which the present application is a continuation in part to insert between superimposed emulsion layers intermediate layers which withstand certain kinds of developers and treating baths but are permeable by others or which can be made permeable by treatment, for instance by saponification.

This device of using variable intermediate layers may be used for the production of a new kind of exposure material which, in the technique of exposure does not differ from the simplicity of the known bi-pack but yields, however, three-color components in a simple manner. This invention consists in a process which uses, in its simplest form, two films, layer to layer travelling through the camera, of which films one carries a single emulsion layer and the other two superimposed emulsion layers, the latter being separated by an intermediate layer of the above kind which may also serve as a filter layer. Instead of two films a single one may be used which carries three superimposed layers, each separated from the other by an intermediate layer of the above kind, which, if desired, may also serve as filter layers.

The essence of the invention resides in the fact that individual layers are treated in such a manner that it is possible to obtain separately the component color pictures from the material. Two courses are possible. In the first, after exposure, which may occur in an ordinary cinematograph camera, first the top layer of the two or three superimposed layers is developed in a developer which leaves unaffected the under-lying intermediate layer and in consequence also the emulsion layers under-lying that intermediate layer. After this first component color picture has been developed the undeveloped silver halide may be removed from the layer by fixing. This fixing is not, however, absolutely necessary. Then, if desired, after drying the layer, the black-and-white image in the upper layer is copied on an auxiliary film by means of light of a color for which the still undeveloped layer or layers of the film is or are not sensitive. After this first

component color picture has been in this manner preserved the first developed layer is mechanically or chemically removed and then the under-lying layer is developed after the hitherto separating layer has been made permeable in a separate bath or simultaneously in the developing operation. This component picture produced in the second layer is printed in the manner described above to produce the second color component picture or is used directly. In case of a bi-pack the third color component picture is in the second film carrying a layer on one side only. If, however, a bi-pack is not used, but only a single film having three superimposed emulsion layers there must be also used for the development of the second component picture a developer which does not attack the separating layer lying between the second and the third emulsion layers. From the second component picture in such a three-layer film there is made a copy on an auxiliary film.

The second course for obtaining the component pictures separates the components produced in the several layers, not by successive copyings but by the difference in their spectral properties. In this procedure one may, for instance, tone the top layer after the development or one may develop by means of a developer which immediately or after separation of the silver image yields a color picture by the process of color development or by the silver anti-diazotate process. Then, in the manner described above, the intermediate layer is made permeable. The under-lying layer is developed and toned in another color. This coloring need not have any relationship with the color of the color component to which the layer in question belongs, but may be dependent only on the process according to which the component pictures of the multi-color copy are to be obtained.

The following example when taken with the accompanying self-explanatory drawing, Fig. 1 of which shows a bi-pack raw film and Fig. 2 of which depicts the processing thereof, illustrates the invention:

A bi-pack is used in which the front film carries two layers separated by an intermediate layer which is impermeable to an acid developer. The layer next to the film is sensitive only to blue light, the superimposed layer is sensitive to green light and is protected from the effect of blue rays by a yellow coloring of the whole layer or by a yellow coloring of the intermediate layer. The rear film is a panchromatic or red-sensitive film and is protected from the access of false light in

known manner by a red filter layer. Moreover, it is preferable to provide anti-halation by a non-actinic coloring of the film support. The exposure in the camera is as usual, the layers being towards each other. After the exposure the rear film is developed in the usual manner; the front film is developed by an acid developer, for instance by the known ferrous oxalate developer whereby a picture is produced only in the top layer. After development the image is fixed. However, this fixing may be omitted without affecting the process.

The green component thus produced in the top layer is now copied with the aid of light lacking blue on an intermediate film sensitive to green or red light, whereby a positive or if desired a reversal negative is obtained which may be used as the second of the components for producing a color picture. The original negative in the top layer is removed with the aid of hot water mechanically or by means of a solvent for silver chemically. Then follows the development of the second blue-sensitive layer with the aid of an alkaline developer which is capable of passing through the previously impermeable intermediate layer. All three component color pictures have now been produced separately for the copying process.

If there has been used for the exposure a film carrying three layers, two intermediate layers are required and these may be permeable for solutions of different pH-value as described in U. S. Patent 2,210,146. If, for instance, the upper intermediate layer is only permeable for alkaline developers, the lower is permeable only for acid developers. First the upper emulsion layer is developed by means of the ferrous oxalate developer which does not penetrate the first separating layer and the intermediate positive is obtained, then this separating layer is made permeable by an alkaline intermediate bath or the second emulsion layer is developed in an alkaline developer which cannot penetrate the second separating layer. Finally the acid developer is again used, whereby the second separating layer is made permeable and the third emulsion layer developed.

What we claim is:

1. A process of producing photographic color component pictures which comprises exposing a bi-pack consisting of a single layer rear film and of a front film carrying two differently optically sensitized silver halide emulsion layers separated by an intermediate layer which is impermeable for certain developers, developing the upper layer of the front film with a developer to which the

intermediate layer is not permeable, copying the developed silver image by means of light which is non-actinic to the still undeveloped layer, removing the upper layer, treating the intermediate layer in a medium which renders it permeable to the following developer; developing the lower layer and printing the developed silver image.

2. A process of producing photographic color component pictures which comprises exposing a bi-pack consisting of a single layer rear film and of a front film carrying two differently optically sensitized silver halide emulsion layers separated by an intermediate layer which is impermeable for certain developers, developing the upper layer of the front film with a developer to which the intermediate layer is not permeable, copying the developed silver image by means of light which is non-actinic to the still undeveloped layer, removing the developed silver image, developing the lower layer with a developer to which the intermediate layer is permeable and printing the developed silver image.

3. A process of producing photographic color component pictures, which comprises exposing a multi-layer film, the single silver halide emulsion layers of which are differently optically sensitized and separated by intermediate layers impermeable for certain developers, in such a manner that each single emulsion layer obtains a component image, developing the uppermost emulsion layer with a developer which is unable to penetrate the underlying intermediate layer, printing the silver image of said developed layer on a suitable photographic material, removing the uppermost emulsion layer, making permeable the intermediate layer and developing the second emulsion layer, and repeating the same operations for the following layers.

4. A process of producing photographic color component pictures, which comprises exposing a multi-layer film, the single silver halide emulsion layers of which are differently optically sensitized and separated by intermediate layers impermeable to certain developers, in such a manner that each single emulsion layer obtains a component image, developing the uppermost emulsion layer with a developer which is unable to penetrate the underlying intermediate layer, printing the silver image of said developed layer on a suitable photographic material, removing the silver image, making permeable said intermediate layer, developing the second emulsion layer and repeating the same operations for the following layers.

JOHN EGGERT.  
GERD HEYMER.